

# UNITED STATES PATENT OFFICE.

KNIGHT E. ROGERS, OF SOUTH MANCHESTER, CONNECTICUT.

## TOBACCO PRODUCT AND PROCESS OF MANUFACTURING THE SAME.

No. 888,743.

Specification of Letters Patent.

Patented May 26, 1908.

Application filed June 7, 1906. Serial No. 320,659.

To all whom it may concern:

Be it known that I, KNIGHT E. ROGERS, a citizen of the United States, residing at South Manchester, in the county of Hartford and State of Connecticut, have invented certain new and useful Improvements in Tobacco Products and Processes of Manufacturing the same, of which the following is a specification.

10 This invention relates to a process of manufacturing tobacco-sheets or boards, and to the product of said process, which product may be utilized for various purposes, although primarily designed for use in the manufacture of tobacco-boxes or other receptacles where it is desired to preserve the odor of tobacco.

In carrying out the improved process, tobacco-stems, stalks, or other tobacco-refuse are severed into small pieces by any desired means, for instance, an ordinary rag-cutting machine, and this tobacco-waste is then placed in a boiler or digester, commingled with chemicals, if necessary, and is thoroughly macerated. From this digester the mass is next placed in a beating or refining-engine, and the fibers thereof are broken up into very small particles or filaments ready for the subsequent steps of the process. At this stage, a certain amount of other fibrous material, which has already been beaten so that the fibers will properly mix with the tobacco-fibers, is added to the mass, this extra material serving to strengthen or harden said mass, and, according to the amount of fibrous material added, being governed by the result sought to be obtained in the finished product. Pulp from tobacco-waste if used alone would produce a soft or "punky" product, but by incorporating therewith vegetable-fibers, such as those of cotton, linen, wood, jute, sisal or other substance the desired degree of hardness in the product may be obtained.

45 While the materials are being commingled in the manner described, any desired flavoring extract, for instance, that of tobacco, may be added, and the mass may be sized to make it waterproof, or it may be loaded with 50 clays to make it dense. In other words, the mixing or incorporating with the mass of different materials should be accomplished at this stage of the process.

From the beating and commingling machine, the pulp is carried to ordinary paper-

making apparatus. If the pulp is submitted to a Fourdrinier machine the product will be thin, and when thick paper or paper-board is required it should be run through a cylinder-machine. In the next stage of the process the product is dried in any suitable manner to expel all moisture, and, finally, it is run through calender-rolls to impart a smooth and finished appearance to the same.

While vegetable fibers, especially those of cotton or linen, are deemed preferable for hardening and strengthening purposes, leather-scrap or other animal material may sometimes be employed for accomplishing these results.

In the manner described a tobacco-sheet or board of any degree of hardness desired, and having and retaining the odor of tobacco, may be manufactured, and this product may be utilized in various ways. If of the thickness of paper-board, boxes or receptacles of various kinds may be manufactured from it, and these boxes will have a tobacco-odor, and will be useful for holding various articles, particularly tobacco-products, such as cigars, chewing-tobacco, snuff, &c.

My invention is not limited to the exact procedure set forth, nor to a product of any especial degree of thickness.

Having thus described the invention what I claim is:

1. The process of manufacturing a tobacco-product consisting of first macerating tobacco, then adding thereto fibrous material, then commingling therewith tobacco-liquor; and finally expressing the moisture and forming the mass into a product of the desired degree of thickness.

2. As an article of manufacture, a tobacco-product composed of tobacco-pulp, and fibrous material, commingled and treated with tobacco liquor in the manner, substantially as described.

3. As an article of manufacture, a tobacco-sheet or board composed of pulp made from tobacco-refuse commingled with fibrous pulp and a flavoring-extract in substantially the manner described.

In testimony whereof I affix my signature in presence of two witnesses.

KNIGHT E. ROGERS.

Witnesses:

LOUIS ST. C. BURR,  
THOMAS JONES.